

1

2,943,917

## PROCESS FOR THE CONVERSION OF HYDROGEN

Daniel H. Weitzel, 3040 Ash Ave., Boulder, Colo., and William V. Loebenstein, 8501 Sundial Drive, Silver Spring, Md.

No Drawing. Filed Dec. 20, 1956, Ser. No. 629,471

14 Claims. (Cl. 23—210)

The invention described herein may be manufactured and used by or for the Government for governmental purposes without payment to us of any royalty thereon.

This invention relates to catalysis and, more particularly, to the catalytic reorientation of ortho- and para-hydrogen.

Hydrogen is, of course, a diatomic molecule and it has been known for some time that this molecule exists in two forms: namely, ortho-hydrogen and para-hydrogen. These two forms are characterized and differentiated from one another by the relationship that exists within the nuclei of the atoms that form the molecule. Each of the atoms has within its nucleus a force or field which can be mathematically described as though caused by a charged particle spinning around in a definite orbital pattern; however, the relationship between these orbital patterns or nuclear spins of the two atoms that form the hydrogen molecule may be different as the particles may be described as rotating either in the same direction or in opposite directions. If the particles that make up the nuclei of the two atoms are rotating in the same direction, the molecule is identified as an ortho-hydrogen molecule; whereas, if the particles in the nuclei are orbiting in directions opposite to one another, the molecule is denominated a para-hydrogen molecule. At this point it should be mentioned that the spin orbits of the two atoms in a given molecule of hydrogen are always parallel although they may rotate in different directions, as aforementioned.

Ortho-hydrogen and para-hydrogen molecules co-exist with one another and have a definite equilibrium relation at a given temperature wherein a fixed ratio of ortho- and para-hydrogen is present; however, this ratio varies widely at different temperatures. For example, at room temperature so-called "normal hydrogen" at equilibrium contains 75% ortho-hydrogen and 25% para-hydrogen; whereas, the equilibrium state of hydrogen at 20° K. is such that 99.8% para-hydrogen and only 0.2% ortho-hydrogen is present.

Now, this fact becomes extremely important in the liquefaction of hydrogen for the following reasons. If we start with normal gaseous hydrogen (75% ortho-) at room temperature and, of course, at equilibrium, it will be in an unstable energy condition when it reaches the temperature of 20° K. at which it liquefies if the liquefaction is carried out rapidly in the customary manner. The hydrogen will, therefore, change or convert slowly from the unstable, high energy state to the stable, low energy level of equilibrium at 20° K. This conversion or reorientation of the nuclei of the ortho-molecules to para-molecules until 99.8% para-hydrogen is present is a highly exothermic energy reaction that causes a substantial volume of the liquid hydrogen to boil off due to the heat liberated. For example, tests have shown that if normal hydrogen (75% ortho-) is quickly liquefied so that little or no reorientation or conversion takes place during the liquefaction process and the liquid hydrogen is stored in a perfectly insulated vessel at about

2

20° K., nearly one-fifth of the original liquid volume is lost and converted to the gaseous state during the first 24-hour period due to the exothermic energy reaction that takes place as the hydrogen slowly changes to the equilibrium energy condition. It will become apparent, therefore, that the liquid hydrogen must be stored in a state of stable energy equilibrium if this rapid boiling away and depletion of the liquid is to be prevented. Actually, in accordance with the equilibrium conditions

5 at 20° K., this means converting normal hydrogen to substantially pure para-hydrogen either during the liquefaction process or immediately after while low temperature refrigeration is still available to carry off the heat of conversion liberated by the exothermic reorientation 10 energy reaction. Normally, however, this exothermic energy reaction that reorients the spin-orbits of the atoms in the hydrogen molecules proceeds much more slowly than the liquefaction process by which the hydrogen gas is liquefied. Therefore, it would be highly advantageous 15 to catalyze this reorientation reaction so that the hydrogen would be in a state of stable energy equilibrium at the time it becomes liquefied or shortly thereafter; or, in other words, have the product of the liquefaction process 20 nearly pure para-hydrogen.

25 Previous attempts to catalyze the foregoing energy reaction have met with a measure of success; however, the reaction was still quite slow, large quantities of the catalyst were required and relatively large liquefier components were needed for a given production rate due to 30 the space requirements of the catalyst. The most effective of the prior art catalysts was a bed catalyst placed in the liquefier reservoir and composed of Cr<sub>2</sub>O<sub>3</sub> on alumina pellets. The catalyst bed was immobilized by placing it under a coarse heavy filter. Liquid hydrogen 35 was fed from the expansion valve of the liquefaction unit, filtered through the catalyst bed and, finally, delivered to a storage Dewar through a transfer siphon. Using approximately 65 liters of about 20% Cr<sub>2</sub>O<sub>3</sub> on a bed of 1/8- by 1/8-inch alumina pellets, a conversion to 95-97% 40 para-hydrogen at a production rate of 240 liters of liquid hydrogen per hour was achieved.

It has now been found, however, in accordance with the present invention that an unsupported ferric oxide gel provides a much more efficient and greatly improved 45 catalyst for both the ortho-para and para-ortho conversion of hydrogen in either the liquid phase or vapor phase condition.

The principal object of the present invention is, therefore, the provision of a new and superior catalytic agent 50 for both the liquid and vapor phase conversion of ortho- to para-hydrogen and para- to ortho-hydrogen.

Another object of the invention is to provide a catalyst 55 for the reorientation of ortho- and para-hydrogen that is approximately forty times as efficient and effective as Cr<sub>2</sub>O<sub>3</sub> on alumina pellets.

A further object of the invention is to provide a novel process for the reorientation of ortho- and para-hydrogen to produce an equilibrium condition.

60 Other objects of the invention are to provide a hydrogen conversion catalyst that requires considerably less space in the liquefaction unit, one which is relatively simple to prepare and activate, a catalyst that is inexpensive and one which can be stored for long periods of time without harmful deterioration.

65 Additional objects of the invention will be in part apparent and in part pointed out specifically hereinafter as the description proceeds.

The ferric oxide gel that comprises the subject matter 70 of the claimed invention is produced by precipitation from an aqueous solution of a soluble ferric salt with a soluble hydroxide. The resultant precipitate usually takes the form of a brown gelatinous substance com-

posed of extremely minute particles although its color may vary from red to almost black. The low solubility of  $Fe_2O_3$  in water produces an enormous supersaturation preceding precipitation which is quite favorable to the formation of a precipitate having minute particles and a large surface area. These particles orient themselves into an enmeshing network that entrains water and constitutes the gelatinous precipitate. This bulky brown gel loses water gradually on standing and becomes more compact. The precipitate must be washed with water until most of the anion of the original ferric salt has been removed; however, washing of the precipitate until approximately 0.1% of the original solution remains, has been found sufficient. After the precipitate has been washed it is filtered and dried. Thereafter, the dried precipitate is crushed and graded through sieves to obtain the desired range in particle size. In this form the precipitate may be stored over extended periods in ordinary glass jars until needed. Immediately prior to use, however, the catalyst must be activated by heating it to a temperature of between approximately 110 and 120° C., preferably in a drying oven, for 12 to 16 hours at a pressure of about one mm. Hg or less. The vacuum should be broken with pure hydrogen gas while the catalyst is still hot.

Repeated tests with ferric oxide gel as a catalytic agent in the conversion of ortho- and para-hydrogen have been performed by one of the inventors at the National Bureau of Standards Cryogenic Engineering Laboratory and have resulted in the conversion of liquid normal hydrogen (75% ortho-) to 5% ortho-hydrogen and less at rates of approximately 2000 S.T.P. liters per minute (2.6 liquid liters per minute) per liter of catalyst used, or 156 liquid liters per hour per liter of catalyst. These results show ferric oxide gel to be approximately 40 times as effective as  $Cr_2O_3$  on alumina pellets when measured under the same conditions.

Tests performed by one of the inventors at the aforementioned laboratory have also resulted in the conversion of 99.8% para-hydrogen to essentially the equilibrium ortho- to para-hydrogen ratio at temperatures ranging from 80° K. to 225° K. The rates of reconversion of para-hydrogen have in these tests been especially high in the temperature region of 80° K. to 140° K. For example, at 100° K. a feed of 99.8% para-hydrogen was converted to within two percent of the equilibrium (38.5% para-hydrogen) concentration at the rate of about 250 S.T.P. liters per minute per liter of catalyst. This property, consisting of the ability to catalyze the endothermic reconversion of para-hydrogen to ortho-hydrogen, points to an important application which has not previously been mentioned, i.e., utilization of the para- to ortho-conversion as a heat sink or source of refrigeration. Thus a quantity of the hydrous ferric oxide suitably placed in tubes in the insulation surrounding a container of liquid para-hydrogen could, by para- to ortho-conversion of the boil-off para-hydrogen vapor, effectively cool a radiation shield attached to the tubes and thereby considerably reduce the heat leak to the remaining liquid in the storage vessel.

Particle size has also been found to have a decided influence on the effectiveness of the hydrous ferric oxide gel in the ortho-para conversion. In general, the effectiveness of the catalyst falls off rapidly when the particle size exceeds that which will pass through a 20-mesh screen. Samples made up of particles ranging from 30 to 50-mesh, however, exhibited about the same activity as samples composed of 50 to 100-mesh particles. There seems to be little advantage in using material finer than 100-mesh as problems arise in connection with containment of the catalyst and the pressure drop across the bed which overbalances the small increase in activity.

At this point it should be mentioned that the catalyst is not ferric hydroxide as the amount of water in the gel varies over wide limits and, therefore, bears no

stoichiometrical relation to the ferric oxide. Also, the catalyst is not a hydrate as the ferric oxide exhibits no tendency to retain any fixed quantity of water. It is felt, therefore, that the dense brown ferric oxide precipitate merely traps or entrains varying amounts of water and is, accordingly, properly denominated "moisture containing ferric oxide."

Another point is that tests have shown the gel breaks down and becomes ineffective as a catalyst if activated at temperatures somewhere between 140° C. and 200° C.; therefore, 140° C. should be considered the maximum activation temperature.

The mechanism by which ferric oxide accomplishes the catalytic reorientation of ortho- and para-hydrogen is believed to depend upon two unsuspected, but important, properties which will now be described.

The first of these properties is the high magnetic susceptibility of the minute gel particles and the attendant tremendous magnetic field gradient confined to a space of the order of the size of the molecule itself. Basically, each ferric oxide gel particle is, in itself, a minute, but powerful magnet. The form of the gel is such that it provides a tremendous surface area having a very porous cellular structure giving the hydrogen molecules a large interface with which to come in contact. The force of the magnetic field around a particle of the catalyst diminishes in intensity very rapidly as the distance therefrom increases; thus, a hydrogen molecule passing in close proximity to the catalyst particle may have one atom greatly affected by the magnetic field while the other atom remains in a much weaker portion of the field even though the two atoms are extremely close to one another. The magnetic force field will, therefore, act to turn only one of the atoms and cause it to flip over and reorient itself into the more stable energy condition. This mechanism is effective to re-align the hydrogen atoms from the ortho-relation to the para- or vice versa depending, of course, upon which condition is the more stable energy state.

The second important property of the ferric oxide gel catalyst is its ability to disassociate the hydrogen molecule and adsorb individual atoms on its surface. This property of the catalyst may be referred to as "activated adsorption." When disassociation of the molecules takes place and atoms of hydrogen are adsorbed on the surface of the ferric oxide particles, these adsorbed atoms will recombine with other disassociated atoms in the stable energy relation. Thus, the catalyst provides a second mechanism that is effective to re-align the spin-orbits of the hydrogen atoms into an equilibrium condition irrespective of whether the conversion is ortho-para or para-ortho.

The use of any catalyst to effect an equilibrium conversion of ortho- to para-hydrogen during the process of liquefaction, of necessity, causes a reduction in the production rate of the liquid hydrogen when compared with a liquefaction process in which no attempt is made to reorient the molecules, as part of the refrigeration capacity of the liquefier must be used to carry off the exothermic heat of conversion. The claimed catalyst, however, in so far as the conversion reaction is concerned, is many times more effective and active to bring about the desired reorientation than the prior art catalysts for this purpose. Therefore, the production rate of liquid para-hydrogen is primarily limited by the refrigeration capacity of the liquefier and not the catalyst which in small quantities is sufficient to bring about the conversion more rapidly than the refrigeration unit can carry off the heat liberated thereby. The  $Cr_2O_3$  on alumina catalyst, on the other hand, must be present in relatively large quantities to cause the required conversion at a given production rate and it thus becomes a limiting factor in those liquefaction units wherein space for the catalyst is limited because, if the unit cannot accommodate the amount of catalyst needed for the conversion at said production

rate, the production rate must be reduced to that which can be handled by the catalyst.

The particle size of the catalyst is not a particularly critical factor if maintained within reasonable limits as many different mesh sizes will bring about the desired end results; however, judicious selection of the particle size will improve the activity and rate of energy reaction and such selection will depend to a large extent on the particular liquefaction apparatus used. For example, in equipment wherein a large drop in pressure across the catalyst bed can be tolerated and still produce the desired production rate, an extremely finely divided form of the catalyst can be used. On the other hand, if the pressure drop is critical, a coarser form should be selected even at the sacrifice of some catalytic activity. The particle size chosen is also somewhat dependent on whether the conversion is to be carried out in the liquid-phase or vapor-phase as obviously, the vapor-phase permits the hydrogen to permeate the catalyst bed much more easily and thoroughly. The foregoing considerations, however, are well within the skill of the art.

Having thus described the several useful and novel features of the catalyst and catalytic reaction for the ortho-para and para-ortho conversion of hydrogen, it will be seen that the many useful objects for which they were designed have been achieved. We realize, however, that certain changes and modifications may occur to those skilled in the art which are within the broad teaching of the instant invention; hence, it is our intention that the scope of protection afforded hereby shall be limited only in so far as said limitations are expressly set forth in the appended claims.

What is claimed is:

1. The process for catalytically converting hydrogen to an equilibrium energy state within the temperature range of from about 20° K. to about 240° K. which comprises passing the hydrogen through a porous bed of heat-activated ferric oxide gel particles.

2. A process as set forth in claim 1, wherein the ferric oxide gel particles are of a size which will pass a 20 mesh screen and the particles are activated by heating to a temperature within the range of from about 110° C. to about 140° C.

3. The catalytic process for converting a mixture of ortho-hydrogen and para-hydrogen in an unstable energy state into an equilibrium energy condition within the temperature range of from about 20° K. to about 240° K. which comprises passing the unstable mixture through a porous bed of heat-activated ferric oxide gel particles.

4. The catalytic process for increasing the ratio of para-hydrogen to ortho-hydrogen in a mixture thereof within the temperature range of from about 20° K. to about 240° K. which comprises lowering the temperature of the mixture, passing said mixture through a finely-divided heat-activated bed of ferric oxide gel, and removing the exothermic heat of reaction.

5. The catalytic process for increasing the ratio of ortho-hydrogen to para-hydrogen in a mixture thereof within the temperature range of from about 20° K. to about 240° K. which comprises raising the temperature of the mixture, passing said mixture through a finely-divided heat-activated bed of ferric oxide gel, and adding heat to replace the heat taken up by the endothermic reaction.

6. A process as set forth in claim 3, wherein the ferric oxide gel particles are of a size which will pass a 20 mesh screen and the particles are activated by heating to a temperature within the range of from about 110° C. to about 140° C.

7. A process as set forth in claim 4, wherein the ferric

oxide gel particles are of a size which will pass a 20 mesh screen and the particles are activated by heating to a temperature within the range of from about 110° C. to about 140° C.

5 8. A process as set forth in claim 5, wherein the ferric oxide gel particles are of a size which will pass a 20 mesh screen and the particles are activated by heating to a temperature within the range of from about 110° C. to about 140° C.

10 9. The catalytic process for converting a mixture of ortho-hydrogen and para-hydrogen at a temperature within the range of from about 20° K. to about 240° K. and below that at which said mixture is stable to a new mixture in a condition of stable energy equilibrium at 15 said temperature which comprises passing the unstable mixture through a finely-divided heat-activated bed of ferric oxide gel particles while removing the exothermic heat of conversion therefrom.

10 10. The catalytic process for converting a mixture of 20 ortho-hydrogen and para-hydrogen at a temperature within the range of from about 20° K. to about 240° K. and above that at which said mixture is stable to a new mixture in a condition of stable energy equilibrium at 25 said temperature which comprises passing the unstable mixture through a finely divided heat-activated bed of ferric oxide gel particles while adding heat to maintain the temperature and replace the endothermic heat of conversion.

11 11. A process as set forth in claim 9, wherein the ferric 30 oxide gel particles are of a size which will pass a 20 mesh screen and the particles are activated by heating to a temperature within the range of from about 110° C. to about 140° C.

12 12. A process as set forth in claim 10, wherein the 35 ferric oxide gel particles are of a size which will pass a 20 mesh screen and the particles are activated by heating to a temperature within the range of from about 110° C. to about 140° C.

13 13. The catalytic process of converting a mixture of 40 ortho-hydrogen and para-hydrogen in an unstable energy-state to an equilibrium energy condition at a temperature within the range of from about 20° K. to about 240° K. comprising the steps of activating a finely divided ferric oxide gel by heating said gel particles to a temperature within the range of from about 110° C. to about 140° C. 45 in a vacuum and passing the unstable mixture through the thus activated ferric oxide gel particles while out of contact with the atmosphere.

14 14. A process as set forth in claim 13, wherein the gel 50 particles are of a size which will pass a 20 mesh screen and the passage of the unstable mixture through the ferric oxide gel particles is commenced while said gel particles are still hot with the vacuum being broken by the passage of said mixture therethrough.

#### References Cited in the file of this patent

#### UNITED STATES PATENTS

|           |               |                |
|-----------|---------------|----------------|
| 370,511   | Wigg et al.   | Sept. 27, 1887 |
| 1,008,321 | Gill          | Nov. 14, 1911  |
| 1,812,527 | Gross et al.  | June 30, 1931  |
| 1,821,195 | Woodhouse     | Sept. 1, 1931  |
| 1,904,439 | Freyermuth    | Apr. 18, 1933  |
| 2,110,240 | Roelen et al. | Mar. 8, 1938   |
| 2,465,235 | Kubicek       | Mar. 22, 1949  |

#### OTHER REFERENCES

Grilly: Atomic Energy Commission, AECU-2245, November 1952.